

J. C. KING.

ELECTRODE.

APPLICATION FILED OCT. 9, 1917.

1,312,260.

Patented Aug. 5, 1919.



*Inventor*  
Jesse C. King

*By*  
*Johnston, Haught & Co.*  
*Attnys.*

# UNITED STATES PATENT OFFICE

JESSE C. KING, OF MONTREAL, QUEBEC, CANADA.

## ELECTRODE.

1,312,260.

Specification of Letters Patent. Patented Aug. 5, 1919.

Application filed October 9, 1917. Serial No. 195,578.

To all whom it may concern:

Be it known that I, JESSE C. KING, a citizen of the United States, and resident of the city of Montreal, in the Province of Quebec and Dominion of Canada, have invented 5 certain new and useful Improvements in Electrodes, of which the following is a full, clear, and exact description.

This invention relates to improvements in 10 electrodes for use in electric furnaces and the like.

It is well known that electrodes which usually consist of carbon waste or burn away quite rapidly at points remote from the active 15 end, thus reducing the efficiency and life of the electrode. The carbon body becomes heated to very high temperatures for a considerable distance back from the end, and this heating renders the carbon more or less 20 readily combinable with oxygen of the air or with other gases, with the result that the electrode burns away, thus reducing the sectional area and consequently altering the resistance and conductivity of the electrode.

25 The main object of my invention is to provide an electrode having on the outer surface thereof a thin coating of non-oxidizing material designed to protect the body of the electrode from combination with gases

30 at all parts of the surface not in actual operation. I have found that a coating of finely ground bauxite is very suitable for this purpose, and the coating may be applied in the manner described in my copending application, Serial No. 99,104, filed May 22nd, 1916. After the application of the protective coating, the electrode is preferably baked, so 35 that the core and the coating become for all practical purposes integral.

40 Referring to the drawing, which represents a cross sectional view of the electrode with the coating applied thereto, 11 designates the core or electrode proper of carbon having the surface 12 roughened by any 45 suitable means. The coating of bauxite 13 is then applied to the roughened surface,

preferably in a plastic condition. The electrode is then baked to drive off the moisture and gases, and to harden both the core and the coating. The bauxite which is ground 50 to a suitable fineness may be molded, pasted, pressed or sprayed on to the roughened carbon core, and when suitably hardened, this coating forms an impenetrable coating between the electrode and the gases of the furnace. If it is desired to mold the surface 55 coating onto the carbon electrode, the latter may be used in a suitable mold as a core and the surface coating may be pressed into the mold around the core in the usual manner. 60 If the surface coating is to be pasted onto the core, a trowel or other suitable implement may be used and this surface coating in plastic condition may be pasted onto the roughened surface of the core, in as even a 65 manner as possible. To spray the coating onto the core, any suitable implement such as a cement gun may be employed.

In some cases, it may be desirable to use a binder consisting of a small proportion of 70 pitch or other carbonaceous bonding material. When a small quantity of such a binder is used, it holds the coating during the baking process where it becomes thoroughly hardened.

Having thus described my invention, what I claim is:—

1. A coating for electric furnace electrodes, consisting of finely ground bauxite and a carbonaceous binder for same. 80

2. An electric furnace electrode comprising a carbon core having a roughened surface, and a coating of bauxite bonded on to the roughened surface.

3. An electric furnace electrode comprising a carbon core having a roughened surface, and a coating of bauxite mixed with a carbonaceous binding material bonded or baked on to the roughened surface. 85

In witness whereof I have hereunto set my 90 hand.

JESSE C. KING.